

Jan. 28, 1958

W. M. DICKSON

2,821,016

METHOD OF HOT FORGING OR EXTRUDING METAL SHAPES  
AND LUBRICANT FOR USE IN HOT FORGING  
AND EXTRUDING OPERATIONS  
Filed March 3, 1955



INVENTOR  
William M. Dickson

BY

*James, Edmund, Morton, Barron & Taylor*  
ATTORNEYS

## 1

2,821,016

**METHOD OF HOT FORGING OR EXTRUDING METAL SHAPES AND LUBRICANT FOR USE IN HOT FORGING AND EXTRUDING OPERATIONS**

William M. Dickson, Houston, Tex.

Application March 3, 1955, Serial No. 491,957

6 Claims. (Cl. 29—424)

My invention relates to improvements in the hot forging of metal articles, and more particularly to the hot forging of steel articles in dies in the presence of a cooling and lubricating solution and to an improved lubricant for use in hot forging or extruding operations.

In high temperature forging operations, as for example in the forging of steel articles or shapes, a number of difficulties have been encountered because of the rapid wear of the dies, even though the billets subjected to forging are previously descaled. One such difficulty, for example, is the scoring of the dies by the hot metal article or shape when it is forced out of the die. This scoring wears the dies and leaves undesirable score marks on the article or shape and gradually increases the size of the die cavity so that it must be discarded. Other difficulties are caused by the hot metal seizing to a part of the die and causing pitting or breakage.

Various attempts have been made to overcome these difficulties by the use of cooling water in and on the dies, but even water or attempts to use oil with water have not avoided the rapid destruction of the dies or eliminated the scoring of the dies and the articles produced therein.

Other difficulties or problems have also developed because of the wear and erosion of the dies in hot forging operations. For example, in the automatic hot forging of nuts and other articles, the wear of the dies, particularly the die cavity increases the amount of metal which must be supplied to the die. However, when additional metal in the form of larger slugs or billets is sent to the dies, difficulties are encountered in the handling of the slugs because of their increased size, which often results in the misplacing of the slugs with respect to the dies by the transfer mechanism.

It has been discovered that when hot steel at a forging temperature, for example upward of 2,000° F., is pressed into a die, there is some tendency of the hot steel to be welded to the die, which is generally of very hard alloy steel. Even though the hot steel is in the die a very short period of time, repeated operations cause heat check marks in the dies along with drag or score marks.

The foregoing difficulties cause rapid wear or destruction of the dies and result in unsatisfactory forgings and in making the operation unduly expensive because the worn dies must be replaced by new dies before a reasonable number of pieces have been produced.

The primary object, therefore, of my invention is to provide an improved method of hot forging or extruding metal articles by which the die life of the forging dies is greatly increased.

Another object of my invention is to provide an improved method of hot forging steel articles including an improved method of lubricating and cooling the forging dies.

Another object of my invention is to provide an improved lubricating and cooling medium for use in high-temperature metal forging and extruding operations.

## 2

In accordance with my invention, the foregoing and other difficulties are overcome and a greatly extended die life is obtained by carrying out the forging operation in the presence of a lubricating and cooling medium comprising a water solution containing suspended colloidal graphite and a soluble oil, which medium is applied to all parts of the forging equipment engaged by the hot billets or slugs delivered thereto for forging and which are forged therein.

- 5 10 In a preferred form of the improved method, the cooling and lubricating solution is applied directly on and into the forging dies and onto the hot billets or slugs as they are introduced into the dies.
- 15 The improved cooling and lubricating solution preferably comprises a water solution containing a relatively small percentage of suspended colloidal graphite and from 1½ to about 7% of a soluble oil.

- 20 An important function of the solution in the forging operation is its lubricating characteristics which prevent any adherence of the hot metal being forged to the highly polished surfaces of the forging dies. Repeated tests have shown, however, that a water suspension of colloidal graphite alone will not effect the desired lubrication of the forging dies and prevent scoring and other damage.
- 25 The same is true of a solution of the soluble oil alone in water, in any proportion.

- 30 Since the forging operation is carried out at extremely high temperatures, it has so far been impossible to determine how the combination of the soluble oil and colloidal graphite in water functions to give the improved results. One theory which was thought plausible was that the small proportion of soluble oil in the water solution adhered to the colloidal particles of graphite and was burned on the surface of the hot slugs or billets, or carbonized thereon as molecular carbon to effect a lubricating action between the hot metal being forged and the forging dies. Furthermore, it was considered that to some extent at least there may be a similar molecular deposit or formation of a carbon lubricant on the polished surfaces of the forging dies. The foregoing may account for the gradual loss of soluble oil from the solution.

- 35 40 45 Regardless of whether or not the foregoing theory or theoretical explanation is correct, the use of the improved cooling and lubricating solution has produced exceptional and unexpected results, which has extended the life of the forging dies five fold or more.

- 45 50 55 For example, in a particular automatic hot forging operation, where steel articles were produced in forging dies from hot metal slugs, the die life where water was used as the cooling and lubricating medium was only sufficient for the production of about 30,000 forged articles of A. I. S. I. 1045 steel. However, after the discovery of the improved cooling and lubricating solution and its use in the same forging operation with the same type of dies as many as 175,000 forged articles of commercial quality were produced on a single set of dies.

- 60 65 70 Other features, objects and advantages of the improvements of the present invention are described more in detail hereinafter in connection with the accompanying drawing comprising a diagrammatic or schematic view partly in plan and partly in vertical section.

- 75 While the features of the invention may be used in connection with various types of hot forging and extruding operations, it will be described and illustrated in connection with its use in the hot forging of steel nut blanks. Referring to the drawing, a round steel bar 10 heated to a bright red temperature of approximately 2300° F. is delivered endwise to a cut-off station, including a fixed member 12 and a movable cut-off knife 14, where substantially cylindrical slugs 16 are successively cut from the end of the bar. Each slug is moved from

the cutting station into a press including a fixed member 18 and a movable member 20, which reduces the length of the slug and bulges its periphery as shown by the slug 22. If the hot bar 10 is coated with scale, this will be substantially all cracked off the periphery of the slugs as they are bulged by the movable press member 20. The ends of the slugs will be free of scale because of the cut-off. If the bar 10 is free of scale, it is advantageous to press the slugs to approximately the desired diameter and thickness for insertion into the cavity 24 of a receiving die 26.

The receiving die 26 with its cavity 24 is shaped, for purposes of illustration, to form the exterior surface of the bulged slug 22 into a hex nut shape in cooperation with the movable die member 28 and punch 30. Upon movement of the die member 28 and punch 30, the slug 22 is moved into the die cavity 24 in opposition to a spring biased knock-out pin 32 extending axially through the receiving die 26. The elements 28 and 30 force the plastic metal of the bulged slug into the corners of the die cavity and form an axial punch hole 33. When the elements 28 and 30 are retracted, the knock-out pin 32 actuated by a plunger 34, forces the shaped slug out of the die cavity 24, after which it is moved to a punch-out position to the right where the shaped slug 36 is set over an opening 38 in a punch-out die. A reciprocable punch 40 is actuated to complete the hole through the axis of the shaped slug to produce a nut blank 42 ready for threading. As the punch 40 is retracted, the nut blank 42 is stripped therefrom by a fixed retaining member 44, through which the punch moves.

During the foregoing operations, the equipment is literally flooded with the cooling and lubricating solution referred to above. A supply of this solution 50 is contained in a supply tank 52, preferably located below the surface of the floor 54, on which the forging equipment is mounted. As an example, the forging equipment described above may comprise elements of an automatic hot forging machine mounted on the floor section 54, so that all of the solution sprayed and delivered onto the machine drains onto the floor from which it flows into a small settling tank 56 where scale and other particles readily settle out, the solution then flowing over a weir 58 directly into the tank 52.

Solution to be sprayed and flooded onto the forging equipment is drawn from the tank through a pipe 60 by means of a pump 62 operated by an electric motor 64. The motor 64 is at least a five horse power motor and may be a 7½ horse power motor for use in connection with larger forging machines, and the pump 62 is adapted to deliver a large volume of solution at a pressure of 80 pounds per square inch through a 1½ to 2 inch discharge pipe 66 and connecting branch pipes 68 and 70. Valved delivery pipes 72 leading from the branch pipes 68 and 70 deliver the solution in regulated streams onto all parts of the equipment used for cutting the high heated slugs and processing them in the forging equipment. For example, it will be noted that streams of the solution are flooded over the elements 12 and 14 and the end portion of the bar 10, as well as the elements 18 and 20. Furthermore, the dies and punches are thoroughly flooded so that cooling and thorough lubrication is secured.

In addition to the streams of solution delivered through the delivery pipes 72 onto all parts of the forging equipment and slugs, a relatively large stream of solution is delivered from the branch pipe 68 through a pipe 74 to a slot 76 along the movable plunger 34 for operating the punch-out pin 32. The member 34 includes a bored duct 78, which connects with a bored duct 80 in the pin 32, this latter duct being provided with a plurality of discharge outlets 82, which pour streams of the solution into the die cavity 24 when the pin is in the position shown in the drawing. However, when the pin is pushed back so that its face is even with the bottom of the die cavity, the flow is cut off for an instant, but even during that time at least two streams of the solution are flowing toward

and into the die cavity 24 as well as onto the slug 22, die part 28 and punch 30. Throughout the operation the solution flows directly onto the various surfaces of the slug so that its surfaces are thoroughly lubricated.

Even though the solution flows onto the hot slug in all processing steps, its movement is so rapid that its temperature is not appreciably lowered and never goes below an effective forging temperature of approximately 2100° F. As an example, nut blanks are forged at a rate of from about 60 per minute for 1½ inch nut blanks, to about 220 per minute for 5/8 or ¾ inch nut blanks. Even the final stages of forging the nut blanks will have a temperature of around 2100° F. On the other hand, it is an object of the invention to deliver a sufficient quantity of solution to the forging dies and other equipment handling the hot slugs or shapes to maintain their temperature well below 1000° F., preferably not over 700° F.

In making up the solution 50 for use in the process, a relatively pure water, which is substantially free of solids is preferably employed. If possible, distilled water should be used. The tank 52 is advantageously designed to hold about 1500 gallons so that an adequate volume of solution is always on hand. Whatever quantity of solution is made up, approximately one part of colloidal graphite by weight is mixed with 6000 parts of water. To this mixture is added approximately 2% by weight of a water soluble cutting oil of a well-known type, such as that used as a cutting oil for tapping or threading. A somewhat larger proportion of colloidal graphite may be employed, but the relatively small proportion referred to has been found sufficient. However, the proportion of soluble oil must be within the range of from 1½ to about 7% by weight. 2% of the soluble oil gives ideal results and is slightly above the minimum requirement so that there is no danger of having an insufficient amount present.

The soluble oil being completely or almost completely soluble in water helps to support the colloidal graphite in a suspended state in the solution. However, it is advisable to provide an agitator, such as the agitator 84 in the tank 52 for continuous or intermittent operation to insure a well-mixed solution, although the colloidal graphite in the solution referred to has very little, if any, apparent tendency to settle out. The agitator 84 may be carried on the shaft 86 and driven by a belt pulley 88.

The solution in the tank 52 may be used over and over again but should be checked periodically in the laboratory to see that the soluble oil content does not fall appreciably below 2% by weight, so that additional soluble oil can be added if necessary. As stated above, it appears that a small proportion of the soluble oil is burned out on the hot blanks or billets, and on the surfaces of the dies, particularly the die 26 which may receive more heat than some of the other elements of the forging equipment. The soluble oil clings to and cooperates with the colloidal graphite to cause this material to cling and coat the die surfaces, as well as the hot slugs or shapes to leave a film or particles of graphite. At least a part of the soluble oil is believed to burn or carbonize on these surfaces and hold the graphite thereon. However, since the soluble oil is present in such a minute amount, it does not leave sufficient solid matter to be objectionable. On the other hand, and in any case it increases the lubricating effect because graphite alone in water is ineffective as a lubricant. When the minute proportion of soluble oil coating the graphite particles is baked or changed on the dies or slugs, the colloidal particles of graphite adhere to the die surfaces, thereby providing a lubricant which may include any carbon formed from the oil.

It is possible that the minute films of oil carried by the colloidal graphite particles are, in some way during heating, carbonized to the die surfaces, and adhered thereto so as to give a lubricant which permits the free

movement of the formed article from the die cavity, or the free withdrawal of punches, such as the punches 30 and 40 from the hot billet, slug or blank without the creation of heat marks or scores on the dies or on the surfaces of the formed articles.

In the hot forging and extrusion of slugs or billets in dies, the improved solution of the present invention allows the hot metal to flow freely under pressure to all corners or crevices of the dies with a minimum amount of galling or seizure of the hot metals to the dies.

In making and using the solution, it is very important that the soluble oil ratio not be increased appreciably beyond the proportions given, since a greater proportion of soluble oil, for example, 10% in the solution, reduces the stability of the solution and gives less cooling and lubrication, thereby allowing the dies to become overheated, which results in taking the temper out of the dies, as well as causing the formation of heat check marks, all of which reduces the useful life of the dies.

While extremely finely ground or colloidal graphite from any source may be used in making up the solution, it has been found convenient to utilize an available commercial liquid product containing 10% by weight of colloidal graphite, having the finest particle size dispersed in 1,3-butylene glycol, the liquid product having a density of 8.9 lbs. per gallon. This product is readily diluted or miscible with water and normally sold as a rubber lubricant. Where this dispersion product is used to make up the solution, approximately one part of the graphite dispersion is mixed with 600 parts of water. The solution containing this graphite dispersion and the soluble oil shows no visible tendency to separate or deposit the graphite, but on the other hand, remains substantially uniform for considerable periods of time, so that it is well suited for use in a recirculating system including a relatively large circulating tank and for use over and over again for lubricating and cooling hot dies.

While various soluble cutting oils, known and used generally for use in tapping, threading and other metal cutting operations may be used, it has been found convenient to utilize one of the commercial products sold by various oil companies, for example, the product sold by the Texas Company known as "Soluble C," soluble cutting oil. The soluble cutting oils sold by other oil companies may also be used.

The improved cooling and lubricating solution according to the invention may advantageously include a small proportion approximating from 0.05% to 1% of a wetting agent for increasing the ability of the water solution to wet metals. Any of the well-known wetting agents may be used for this purpose, which are soluble or readily dispersed in water. In fact, the soluble oil itself greatly increases the wetting power of water for metals.

The improved solution of the present invention provides an effective medium for lubricating and cooling dies used in high temperature forging and extruding operations. Its unusual and unexpected action is believed to result in providing an almost invisible coating on the die surfaces and the surfaces of the hot metal billets or slugs being forged or extruded. The effectiveness of the lubricant and method of the invention have been proved in long continuous forging operations at temperatures of from 2100 to 2300° F. and in comparison with other presently used cooling agents and methods.

It is believed that the reason for the ineffectiveness of graphite alone, for example when supplied to hot die surfaces with water, is that the graphite has no tendency

to wet or adhere to the die surfaces but may, in fact, run off or be squeezed out along with the water.

I claim:

1. In the hot forging of steel articles from heated steel bar stock in which the steel bar stock is heated to a temperature approximating 2300° F., slugs are cut successively from one end of the heated steel bar stock by a cut-off means, the slugs being placed in succession in a die cavity of a forming die and pressed therein to the shape of the steel article, the improvement in which a cooling and lubricating composition is flooded over the slugs as they are cut from the bar stock, the cut-off means and all parts of the forming die during the cutting of the slugs and the forming of the steel articles therefrom, said cooling and lubricating composition comprising a water solution consisting essentially of water, approximately one part by weight of finely-divided graphite to 6000 parts by weight of water, and from approximately 1.5 to 7% by weight of a soluble cutting oil, whereby 20 scoring and excessive wear of the forming die is prevented.
2. The improvement as claimed in claim 1, including the provision of a body of the cooling and lubricating composition, continuously passing the composition from 25 the body to the cut-off means and die, returning the composition after flooding the cut-off means and die to the body of the composition for recirculation.
3. In the hot forging of steel articles from heated steel bar stock in which the steel bar stock is heated to a temperature of from 2000° to 2300° F., slugs are cut successively from one end of the heated steel bar stock by a cut-off means, the hot steel slugs being placed in succession in a die cavity of a forming die and pressed therein to the shape of the die, the improvement in which 35 a cooling and lubricating composition is flooded over the slugs as they are cut from the bar stock, the cut-off means and all parts of the forming die during the cutting of the slugs and the forming of the steel articles therefrom, said cooling and lubricating composition comprising 40 a water solution consisting essentially of water initially substantially free of solids, approximately one part by weight of finely-divided graphite in suspension to 6000 parts by weight of water, and approximately 2% by weight of a soluble cutting oil, whereby scoring and excessive wear of the forming die is prevented.
4. A fluid cooling and lubricating composition for cooling and lubricating the dies during the hot forging or extruding of hot metal billets or slugs in the dies, said composition consisting essentially of water, approximately 50 one part by weight of a mixture composed of 10 parts of colloidal graphite and 90 parts of 1,3 butylene glycol to 600 parts by weight of water, and from about 1.5 to approximately 5% of a soluble cutting oil.
5. A fluid cooling and lubricating composition for 55 cooling and lubricating dies during the hot forging or extruding of hot metal billets or slugs in the dies, said composition consisting essentially of a fluid aqueous mixture containing approximately one part of colloidal graphite to approximately 6000 parts by weight of water, and from approximately 1.5 to 7% by weight of a soluble cutting oil.
6. A composition as claimed in claim 5, including a small proportion of a metal wetting agent.

65 References Cited in the file of this patent

UNITED STATES PATENTS

- |           |        |               |
|-----------|--------|---------------|
| 1,428,148 | De Cew | Sept. 5, 1922 |
| 2,588,625 | Ferner | Mar. 11, 1952 |